

June 27, 1933.

H. H. BAILEY

1,915,916

## PROCESS OF COKING HYDROCARBON MATERIAL

Filed May 22, 1929

Fig. 1.



Fig 2.



## INVENTOR

Henry H. Bailey

BY *John D. Lach.*

**ATTORNEY**

## UNITED STATES PATENT OFFICE

HENRY H. BAILEY, OF CHICAGO, ILLINOIS, ASSIGNOR TO THE BARRETT COMPANY, OF NEW YORK, N. Y., A CORPORATION OF NEW JERSEY

## PROCESS OF COKING HYDROCARBON MATERIAL

Application filed May 22, 1929. Serial No. 305,043.

This invention relates to the distillation of heavy hydrocarbon materials and more particularly to the distillation and coking of hydrocarbon pitches and tars. By the term heavy "hydrocarbon materials" is meant material such as coal gas tar, water gas tar, coke oven tar, blast furnace tar, wood tar, pitches derived from the aforementioned tars, petroleum pitches, or any other similar material.

One object of this invention is to distill and coke hydrocarbon materials to obtain a maximum yield of distillate oils and at the same time a coke product of relatively low ash, sulfur and volatile matter content that is also hard, dense and is, therefore admirably suited for metallurgical purposes. Another object is to provide a process for distilling and coking hydrocarbon materials which may be conducted in a retort or still and does not require additional apparatus or equipment for coking the residue remaining in the still after the distillate oils have been driven off therefrom, i. e., does not require refractory brick or fireclay ovens or retorts for the treatment of the residue in the still to form coke therefrom. Another object is to recover volatiles lost in usual beehiving operations.

20 Lunge, 5th Edition, 1916, Part II, "Coal Tar", page 564 et seq., indicates that various attempts have been made to completely distill coal tar and coal tar pitch to obtain a coke residue but that the only methods which 25 have heretofore proved practical involved coking in separate vessels from the stills in which the distillation operation was conducted. In this connection on page 564 he states—"The apparently simplest plan, that 30 of carrying on the process in the tar still itself to the stage of coke, is not feasible. We have seen, on page 397, that cast iron is not well adapted for tar distilling, and wrought iron would be burnt away too quickly. 35 \* \* \* Hence distilling the tar up to pitch in the ordinary stills, and distilling the pitch in separate vessels, either charging them with it in the solid state, or running it while 40 still liquid into the pitch oven, cannot be 45 avoided. The oven may be a brickwork muf-

fle, or a fireclay gas-retort, or an iron vessel of some shape or other".

It has also been proposed to completely distill coal tar in a still mounted or housed in a furnace so that products of combustion 55 from the furnace pass entirely around the sides of the still and about both ends thereof, and to distill coal tar into and through the pitch state to coke as one continuous operation in an internally and externally fired still, the 60 internal firing being accomplished by flues positioned in the interior of the still and arranged to have products of combustion from the furnace pass therethrough. The aforementioned proposals, it will be noted, involve 65 stills of special and intricate construction.

In carrying out this invention a retort or still of usual construction may be utilized. In other words, my process of distilling and coking coal tar pitch or other liquid hydro- 70 carbon material may be practiced in the usual wrought iron or steel stills without danger of destructively overheating or otherwise deleteriously affecting the still. Preferably, however, the retort is slightly modified to 75 provide covered or valve controlled openings in the side of the still remote from the distillate offtake, and a stack over the manhole in the top of the still. The function of the openings and stack will be hereinafter ex- 80 plained.

I have found that a high quality coke low in sulfur and ash and possessing satisfactory mechanical strength may be prepared from hydrocarbon materials such as coal tar pitch 85 while recovering substantially all available volatiles lost in the usual beehiving operations and employing only a simple still, by first subjecting the hydrocarbon material to a preliminary distillation operation in the still 90 to remove the major portion of the available volatiles which will be given off as the result of a simple distillation operation, but leaving in the residue a substantial volatile content, ordinarily not less than about 7% of the 95 residue by weight, and then subjecting the residue while remaining in the still to a beehiving operation by admitting air into the still in carefully controlled quantities to prevent an excessive rise of temperature in the 100

still while igniting the remaining volatiles to cause coking of the mass to take place.

The success of my process may be explained upon the theory that the volatile matter left in the charge after my preliminary distillation is sufficient to cause ready ignition and burning thereof and thus eliminate the heaviest oils which cannot be driven off by external heat and at the same time by controlling the admission of air into the still the heat will not be great enough to damage the still. The low volatile coke which is found next to the still bottom will tend to act as insulation and protect the still bottom from the internal heat.

In accordance with this invention, coal tar pitch or other hydrocarbon material is charged into the retort in either liquid or solid form and is distilled, the distillate passing from the distillate offtake into the usual condensers. Heating of the retort by products of combustion from the furnace in which the retort is housed or by other means is carried on until a semi-coke mass containing ordinarily at least 7% by weight of volatiles forms in the retort. It has been found that more than 30% by volume of the coal tar pitch passes off and is collected as distillate oil, usually for 30 to 40% by volume of the pitch charged into the still being collected before the semi-coke stage is reached.

At this stage of operation, i. e., when a semi-coke has formed in the still and little or no distillate comes off from the mass in the still, steam is passed through the still to remove any vapors therein. The fire in the furnace, or other means employed for heating the still, is shut off before or during the interval steam is passed through the still. The steaming cycle may be of short duration—a few minutes, or if desired steam may be introduced into the still or passed through the pitch for from 4 to 6 hours or more during the period that the still is heated so as to aid in driving off the heavier vapors from the pitch mass in the still. At the termination of the steaming cycle the side openings are uncovered and air or other oxygen-containing gas admitted through these side openings and the stack is placed in communication with the interior of the still to create a draft in the still and cause the products of combustion formed by reaction between the oxygen of the air and a portion of the residue to pass therefrom through the stack into the atmosphere. The volatiles remaining in the residue react with the air or other oxygen-containing gas introduced into the still. In other words, introduction of air or other oxygen-containing gas causes the volatiles remaining in the residue in the still to burn and thus the residue in the still is beehive coked and a dry coke is formed. The term "beehive coked" or "beehive coking" is used herein to describe the action taking place in the still between the air or other

oxygen-containing gas and the residue therein, which action is comparable to that occurring in the coking of material in the usual beehive coke oven.

The air is admitted slowly in regulated quantities, which are determined by the size and number of openings in the sides of the still, to the residue therein so that the beehiving proceeds slowly and excessively high temperatures are not developed in the retort. This beehive coking is allowed to proceed for more than 12 hours, preferably for approximately 36 hours. After the beehiving operation the coke in the still is quenched by means of water introduced thereinto and then the coke is withdrawn from the still through a discharge port provided for this purpose. The coke product thus obtained is of low ash, sulfur and volatile matter content, is dense, hard and admirably suited for metallurgical purposes, much more so than any coke heretofore produced in a still or retort in which the distillation of pitch to coke was performed in one continuous operation.

Accordingly, it will be noted that this invention involves the distillation of hydrocarbon material to drive off distillate oils therefrom and thereafter beehiving the residue in the still to form coke.

For purposes of illustration, I will now describe a specific example of the application of my invention, employing a form of still as shown in the accompanying drawing, in which—

Fig. 1 is a sectional view, some parts being shown in elevation, of a still adapted to practise this invention, and

Fig. 2 is a front elevation corresponding with Fig. 1, of the side of the still remote from the distillate offtake.

In the drawing, 1 indicates a still or retort of the type commonly used in the distillation of coal tar or pitches. This still may be externally heated by products of combustion generated in combustion chamber 16, into which suitable fuel, such as oil or gas, may be introduced through pipe 17 and burned therein. The still has the customary goose neck or distillate offtake 3, communicating with the usual condenser 18. Condensate from the condenser flows to collector 19. A valve controlled charging pipe 2 and a man-hole 4 provided with a cover 9 are positioned in the top of the still. The front of the still is formed with a discharge port or gate controlled opening 8, through which the residue or coke product in the still may be removed.

In accordance with this invention, the side of the still remote from the distillate offtake 5 is provided with a plurality of openings 7 positioned above the usual level of the semi-coke formed in the still after the material therein has been heated in the preliminary distillation operation. Each of the openings 7 is provided with a closure plate 6, or may

have valve or other control means for regulating the extent of opening. Above the level of openings 7, a valved pipe 13 for admission of steam to the retort is provided. 5 The retort is also preferably equipped with a stack 5 hingedly mounted to the side of the manhole 4 in the top of the still, and a valved pipe 10 which terminates near the bottom of the retort midway of discharge pipe 11, the 10 latter having small lateral openings 12. The pipe 11 is preferably arranged close to the bottom of the retort. In Fig. 1 the stack 5 in dot and dash lines is shown in position to create a draft in the retort 1 and in full lines 15 is shown resting on support 14, its position during the distillation operation when manhole 4 is closed by cover 9.

In operation, hydrocarbon material such 20 as coal tar pitch in either liquid or solid form, is charged into the still 1. If liquid, the material is pumped from its source through the charge pipe 2 into the still 1, and if solid the material may be charged into the still through manhole 4. The openings 7, discharge outlet 25 8 and the manhole 4 are closed and the still is then heated by hot products of combustion in combustion chamber 16 in which the still is housed or mounted or by other suitable heating means. The heating is continued 30 until the volatile content has been largely driven off and a semi-coke residue remains in the still as indicated hereinbefore. The stopping point of the distillation operation can readily be determined by an inspection 35 of either the residue in the still or the heavy distillate oils then being collected, or both. If desired, steam may be admitted through pipes 10 and 11 at the commencement of the 40 distillation operation and continued throughout the distillation, thus preventing clogging of the openings 12, as will be more fully explained hereinafter, and assisting the driving off of the volatiles from the hydrocarbon material in the still. The duration of the 45 distillation period is, of course, variable and depends primarily on the amount of the charge and the rate of heat input to the still.

After the distillation has been completed, 50 manhole cover 9 is removed and steam is admitted through pipe 13 and passed through still 1. Heating of the still is discontinued upon completion of the distillation period and after steam has been passed through the still to remove residual vapors therefrom, 55 thus eliminating this explosion hazard, closure plates 6 are removed from openings 7 and air or other oxygen-containing gas is admitted through openings 7 into the still 1. At about the same time the stack 5 is moved 60 about its hinged connection into communication with the interior of the still, as shown in dot and dash lines Fig. 1, thus creating a draft which causes the products of combustion between the air or other oxygen-containing gas and the residue in the still to pass

therefrom through the stack into the atmosphere. This beehive coking of the residue in the still is permitted to continue slowly for a considerable period, 12 hours or more, preferably about 36 hours, until a dense, solid, 70 dry coke is formed. Water is then injected into retort 1, as for example through manhole 4, to quench the coke which is thereafter removed through the discharge port 8. 75

Air or other oxygen-containing gas may be admitted to the interior of the residue during the beehive coking operation through the pipe 11 positioned near the base of the still. When the introduction of air in this manner is desired, clogging of the openings 12 during the distillation operation when the pitch is transformed from liquid to semi-solid coke state may be avoided by passing steam through pipes 10 and 11. 80

According to a preferred embodiment of this invention a charge of 220 to 230° F. melting point coal tar pitch of 3000 gallons was placed in a usual 200 barrel tar still and the still was heated by products of combustion from the furnace in which the still was housed, for eight hours. 30 to 40% by volume of the pitch charged was thus obtained as distillate oil and a semi-coke was formed in the still having a volatile content of from 7 to 10%, by weight. Beehive coking as above described, was conducted for 36 hours resulting in a yield of 8 tons of firm, dense coke having a low ash, sulfur and volatile matter content. 95

Pitch coke when produced in accordance 100 with this invention may be expected to have the following composition:

|                                        | Per cent |
|----------------------------------------|----------|
| V. C. M. (volatile combustible matter) | 2.4      |
| Ash                                    | .8       |
| Sulphur                                | .9       |
| Fixed carbon                           | 96.8     |

In accordance with usual practice in analyzing coke the sulphur content was determined separately and accordingly the results given for the V. C. M., ash and fixed carbon contents include the sulphur present in the coke. This accounts for the fact that the percentages above total 100.9%, the excess 115 .9% representing the sulphur content.

The term "retort" is used in the specification and claims in a generic sense and is intended to include any vessel suitable for the distillation and coking of hydrocarbon material. 120

It will be understood that while a preferred embodiment of this invention has been described herein, various changes in the details thereof might be made and the invention is not to be limited to the disclosure herein but only by the scope of the appended claims. For example, if desired, the still may be externally heated at intervals or continuously 125 while the residue in the still is beehive coked. 130

I claim:

1. The process of coking heavy liquid hydrocarbon material in a retort, which comprises externally heating a mass of said material in said retort until a semi-coke is formed in the retort, discontinuing said heating operation, and then introducing an oxygen-containing gas into contact with the hot semi-coke in said retort to burn volatiles in the semi-coke and thus form a dense coke in said retort.
2. The process of coking coal tar pitch, which comprises externally heating a mass of said pitch in a retort until a semi-coke is formed in the retort, discontinuing said heating operation, and then introducing air into contact with the hot semi-coke in said retort to burn volatiles in the semi-coke and thus form a dense coke in said retort.
3. The process of coking coal tar pitch, which comprises heating a mass of said pitch in a retort until a semi-coke having a volatile content of from 7 to 10% is formed in the retort, discontinuing said heating operation and for more than twelve hours introducing air into said retort to burn a portion of the residue therein and thus form a dry coke in said retort.
4. The process of coking heavy hydrocarbon material in a retort, which comprises heating a mass of said material in said retort until the major portion of the volatiles there-

in is driven off and a pitch residue having not less than approximately 7% of volatiles by weight remains in said retort, and thereafter introducing air to burn the residue in said retort to form coke.

5. The process of coking coal tar pitch in a retort, which comprises heating a mass of said pitch in said retort until the major portion of the volatiles therein is driven off and collected and a pitch residue having not less than approximately 7% of volatiles by weight remains in said retort, and thereafter discontinuing the said heating operation and introducing air into said retort to burn a portion of the residue and form dry coke in said retort.

6. The process of coking heavy hydrocarbon material in a retort, which comprises heating a mass of said material in said retort until the major portion of the volatiles therein is driven off and collected and a pitch residue having not less than approximately 7% of volatiles by weight remains in said retort, steaming said residue to drive off further volatiles therefrom, and thereafter introducing an oxygen-containing gas below the surface of said residue to burn a portion of the residue to form coke in said retort.

In testimony whereof, I hereunto affix my signature.

HENRY H. BAILEY.

35

100

40

105

45

110

50

115

55

120

60

125

65

130